

# UNITED STATES PATENT OFFICE.

ARTHUR ARENT, OF DES MOINES, IOWA.

## PROTECTIVE TREATMENT OF MATERIALS.

1,388,829.

Specification of Letters Patent. Patented Aug. 23, 1921.

Original application filed June 26, 1919, Serial No. 306,928. Divided and this application filed January 29, 1921. Serial No. 441,084.

To all whom it may concern:

Be it known that I, ARTHUR ARENT, a citizen of the United States, residing at Des Moines, in the county of Polk and State 5 of Iowa, have invented certain new and useful Improvements in Protective Treatment of Materials; and I do hereby declare the following to be a full, clear, and exact description of the invention, such as will enable others skilled in the art to which it 10 pertains to make and use the same.

This invention relates to protective treatment of materials and especially to treatment of materials for the purpose of reducing 15 their inflammability; and it relates more particularly to the utilization for this purpose of tarry materials such as creosote, tar or pitch, asphalt, and the like, having incorporated therewith a fire-retardant metal 20 compound, more particularly a metal compound, such as a salt of antimony or the like which is soluble in creosote or the like, alcohol, amyl acetate, tetrachlorid or other chlorid of carbon, or other non-aqueous solvent; and to the resultant products. A 25 metal compound which is insoluble in water and which is decomposed by water with formation of an insoluble compound or compounds is particularly desirable for purposes of the present invention.

I have found that materials such as creosote, tar, asphalt, and the like, which are here designated generically as tarry materials for purposes of convenience, may be 35 rendered more fire-resistant and less inflammable, by incorporating therewith a fire-retardant metal compound of a class typified by compounds of antimony, anhydrous antimony trichlorid being the most desirable 40 representative of this class of compounds at present known to me; and that materials treated with the so modified tarry substances may be rendered non-inflammable. For the sake of a concrete disclosure of the invention, the use of antimony trichlorid will be 45 referred to more particularly hereinafter, but it is to be understood that the invention is not limited to the use of antimony trichlorid, the use of which is here described 50 by way of illustration and not by way of limitation.

In my prior copending application Serial No. 306,928, filed June 26, 1919, of which the present application is a division, I have 55 claimed the treated or modified tarry materials aforesaid and the process of preparing

them. The claims of the present application are directed to processes of employing such modified tarry materials in the treatment of other materials to protect the latter 60 and reduce their inflammability; also to the resultant protected materials and articles of manufacture.

Untreated tarry materials of the type above mentioned are very widely used in 65 the arts, especially in impregnating or coating wood, paper, textile fabrics, roofing, etc., for the purpose of preserving or waterproofing the same. In their untreated condition, such tarry materials inflame readily when heated to a sufficiently high temperature and burn with great vigor; and wood, paper, etc., impregnated therewith are also highly inflammable. According to 70 the present invention, modified tarry materials, prepared as set forth in my prior application aforesaid, are employed to impregnate, coat, or otherwise treat combustible materials, especially fibrous materials, and thereby to render them non-inflammable or 75 substantially so.

Generally speaking, the fire-retardant metal compound employed in practising the present invention may be incorporated directly with the material to be fireproofed, 80 or it may first be dissolved in a suitable solvent vehicle such as carbon tetrachlorid or other carbon chlorid, amyl acetate, or the like, amyl acetate having special advantages for the purposes in view. For example, either crude or refined creosote derived from distillation of either coal or wood, treated by dissolving therein antimony trichlorid in the proportion of 2 pounds to each gallon of creosote, is rendered 85 much less inflammable; and materials such as cloth, paper, wood, etc., to which this treated creosote is applied, are rendered very resistant to fire. When thoroughly impregnated or coated with the preparation, 90 they are rendered non-inflammable. That is, they can be subjected to the direct impingement of a flame without taking fire, even though the flame be directed into contact with the treated material continuously. 95 The material will eventually carbonize but it will not take fire.

Solution of antimony chlorid in creosote may be effected at ordinary temperatures without heating, but moderate heating facilitates solution and is therefore desirable 100 in practice. The amount of antimony tri-

chlorid employed may vary considerably in accordance with the degree of non-inflammability or resistance to fire which it is desired to attain, but the proportions given in 5 the above specific example are found in this particular case to render the creosote and articles to which such treated creosote is applied, non-inflammable in the sense above explained and to be therefore thoroughly 10 satisfactory.

In treating tar, pitch, or asphalt, of the character commonly employed for roofing, the tar is best melted by gently heating, and when it is thoroughly liquefied, antimony 15 chlorid is added thereto with continuous stirring.

The use of antimony trichlorid in the proportion of one part by weight to four parts of the tar, pitch, or asphalt, yields a 20 substantially fireproof product, that is, a product which will not inflame.

As before stated, the antimony chlorid may first be dissolved in a suitable solvent, and then mixed with the material to be fire-proofed. For instance, the necessary amount 25 of antimony trichlorid may be dissolved in amyl acetate, and this solution then mixed with creosote to give a composition of excellent character for impregnation of paper, 30 canvas, or the like; or the mixture may be used, in conjunction with other materials, such as pigments, varnish gums, etc., if desired, by painting it or otherwise applying it as a coating composition to materials or 35 articles of any kind which it is desired to coat or protect. Similarly the amyl acetate or other solution of antimony trichlorid may be incorporated with semi-solid or solid tars, pitches, and asphalts, to give fireproof 40 paints or coating compositions applicable for numerous purposes. All these mixtures confer non-inflammability upon material treated therewith, when antimony trichlorid is present in sufficient quantity; and the degree 45 of non-inflammability or fire-resistance may of course be varied as deemed desirable by varying the proportions of antimony trichlorid used.

The treated products prepared as above 50 described may be applied, when in liquid condition, by brushing, dipping, spraying, etc.; and materials and articles to which such products have been applied are rendered fire-resistant or non-inflammable as 55 already explained and are included within the present invention.

Subjecting articles coated or impregnated 60 with the products above described, to the action of air, and particularly to the action of water, steam or moist air, has the effect of apparently oxidizing the antimony to some extent at least in the exposed outer surfaces or layers with formation of highly fire-retardant basic compounds in the nature of or 65 analogous to basic chlorids or oxychlorids

of antimony, which are insoluble in water and tenaciously adherent, so that the fabric or other article protected with a composition of the character above described does not lose its fire-resistant character even upon 70 prolonged exposure to weather. It is for this reason, among others, that metal compounds which act in this respect similarly to anhydrous antimony trichlorid are especially advantageous in practising the present 75 invention. The special desirability of antimony trichlorid is due to the fact that it is readily soluble in a number of organic solvents miscible with tarry substances, to give solutions or mixtures with which materials 80 can be impregnated or otherwise treated, and also to the fact that it does not dissolve in water and hence cannot be washed out of material treated therewith, but on the contrary decomposes instantly upon contact 85 with water, forming insoluble products above mentioned. Other salts of antimony such as the sulfate are ordinarily less desirable because of the possibility of stronger 90 corrosive action consequent upon development of free sulfuric acid; although this corrosive action may be guarded against in the case of either the chlorid or the sulfate by incorporating an antacid substance such as sodium carbonate, lime, or the like, with 95 the composition or by washing the finally coated or impregnated articles with a mildly alkaline solution of any appropriate character. Neither is the invention restricted in its broader aspects to the use of antimony 100 salts, although antimony salts, and antimony chlorid especially, give in practice results which are markedly superior to even such other metal compounds as react with water in a somewhat similar manner. 105

What I claim is:

1. The process of protectively treating materials which comprises applying thereto a tarry substance having incorporated therewith a suitable proportion of a fire-retardant 110 metal compound which is soluble therein or miscible therewith to form a homogeneous product, said compound having the property of decomposing substantially immediately upon contact with water to yield a water- 115 insoluble product.

2. The process of protectively treating materials which comprises applying thereto a tarry substance having dissolved therein a salt of antimony that is substantially immediately decomposed upon contact with water. 120

3. The process of protectively treating fibrous materials which comprises applying thereto a tarry substance having antimony trichlorid incorporated therewith. 125

4. The process of protectively treating fibrous materials which comprises applying thereto a tarry substance having a fire-retardant hydrolyzable compound of antimony incorporated therewith. 130

5. The process of protectively treating materials which comprises applying thereto creosote having antimony trichlorid dissolved therein in the approximate proportion of two pounds of antimony trichlorid to one gallon of creosote, and thereafter exposing the treated material to moist air. 9. As new articles of manufacture, materials rendered non-inflammable by association with a tarry substance having incorporated therewith a salt of antimony that is substantially immediately decomposed upon contact with water. 35
6. The process of protectively treating fibrous materials which comprises applying thereto a protective composition comprising antimony trichlorid incorporated with tarry material in fluid condition. 10. As new articles of manufacture, materials associated with a tarry substance having antimony trichlorid incorporated therewith. 40
7. The process of protectively treating materials which comprises applying thereto a protective composition comprising antimony trichlorid incorporated with a tarry material in fluid condition in the proportion of about one part of antimony trichlorid to from four to five parts of the tarry material, by weight. 15 45
8. As new articles of manufacture, materials rendered non-inflammable by association with a tarry substance having incorporated therewith a suitable proportion of a fire-retardant metal compound which is soluble therein or miscible therewith to form a homogeneous product, said compound having the property of decomposing substantially immediately upon contact with water 25 to yield a water insoluble product. 50
13. As new articles of manufacture, materials associated with a protective composition comprising antimony trichlorid incorporated with a tarry material in fluid condition in the proportion of about one part of antimony trichlorid to from four to five parts of the tarry material, by weight. 55

In testimony whereof I hereunto affix my signature.

ARTHUR ARENT.